

Sept. 26, 1939.

A. CIMOROSI

2,174,202

FIREWORKS

Filed May 18, 1938

2 Sheets-Sheet 1



**Fig. 1**



**Fig. 2**



**Fig. 3**



**Fig. 4**



**Fig. 5**



**Fig. 6**



**Fig. 7**



**Fig. 8**

INVENTOR  
ALBERTO CIMOROSI.

BY



ATTORNEYS

Sept. 26, 1939.

A. CIMOROSI

2,174,202

FIREWORKS

Filed May 18, 1938

2 Sheets-Sheet 2

FIG. 11.



FIG. 12.



FIG. 13.



FIG. 14.



FIG. 16.



FIG. 15.



INVENTOR  
ALBERTO CIMOROSI.

BY *Alberto CIMOROSI*  
ATTORNEYS.

## UNITED STATES PATENT OFFICE

2,174,202

## FIREWORKS

Alberto Cimorosi, Tippecanoe City, Ohio

Application May 18, 1938, Serial No. 208,623

4 Claims. (Cl. 102—23)

My invention relates to fireworks.

In particular, this invention has to do with a fireworks article which, when ignited, projects a jet of flame.

5 It is an object of my invention to provide a molded, formed pyrotechnical means for forming, when ignited, a jet of flame or smoke. This member is damp as a result of the process of its manufacture and its composition, and it is the object of this invention to provide a method of dehydrating this pyrotechnical member so that it will readily ignite because it is dried quickly.

10 It is a further object to provide such a dehydrated pyrotechnical member with a casing capable of withstanding combustions of the pyrotechnical composition without rupturing so that the smoke and flame may pass out through a vent in the casing through which a fuse has been introduced. This casing is preferably made of a 15 conglomerate as hereinafter described.

15 It is an object to provide a fireworks article such as a rocket having a dehydrated smoke and flame producing composition, the gases from which are ejected through a conglomerate, relatively hard and strong casing to which casing there is attached, preferably by the adhesiveness 20 of the casing, a sky rocket stick.

Referring to the drawings:

Figure 1 is a side elevation of one form of 25 the smoke and flame producing and gas generating composition;

Figure 2 is an end elevation thereof;

Figure 3 is a transverse section taken longitudinally through the completely coated pellet;

30 Figure 4 is a transverse section through the completely coated pellet;

Figure 5 is a section taken longitudinally through the completely coated pellet showing the fuse in position;

35 Figure 6 is a similar view taken transversely of the article with the fuse in position;

Figure 7 is an exterior view of the completely coated pellet with a fuse in position showing the side elevation thereof;

40 Figure 8 is an end elevation thereof;

Figure 9 is a side elevation of the article attached to a stick to make a sky rocket; and

45 Figure 10 is a longitudinal section taken through the completed hard end portion of the stick.

Figure 11 is a front elevation of a spinner embodying this invention.

Figure 12 is a top plan view thereof.

50 Figure 13 is a section on the line 13—13 of Figure 12.

Figure 14 is a side elevation thereof.

Figure 15 is an elevation of a cylindrical body embodying the features of this invention.

Figure 16 is a vertical section therethrough.

It will be understood that the smoke and flame 5 producing and gas generating molded interior member may be either cylindrical or of any other form, such as in the form of a ball, etc.

According to my method, I first mold a conglomerate mixture of charcoal, saltpeter, sulphur, 10 aluminum magnesia powder or powders and any other color producing materials that may be necessary.

This molded body is then subjected to the second step of my process for the purpose of dehydrating it. Great difficulty has been experienced with rockets over long periods of time that remain damp by reason of the fact that the interior composition has been enclosed immediately after making with the casing hereinafter described. 15

Rockets so made would not ignite. Therefore, after the pellets 1 are molded and are ready to be tumbled to apply the conglomerate coating, before this coating is applied, I apply a mixture of silicate of soda, whiting and charcoal which is 20 poured over the pellets. Any desired method of coating them may be employed, such as tumbling, dipping, spraying or brushing. This coating is designated in the drawings as 2. It has the effect of making the pellets dry very quickly and of 25 dehydrating them. It also protects the pellets against the absorption of moisture as a result of the application of the next succeeding coating which forms a hard casing to complete the pyrotechnical device. The proportions of silicate of 30 soda, whiting and charcoal are as follows:

|                       | Per cent<br>by weight |
|-----------------------|-----------------------|
| Silicate of soda..... | 80                    |
| Whiting.....          | 13 $\frac{1}{2}$      |
| Charcoal.....         | 6 $\frac{1}{2}$       |

The next step of the process is to apply the conglomerate coating 3 which may be made from a mixture of glue, wood flour, granular material, 45 sawdust, confetti or aluminum flakes or filter. The pellets 1 with their coating 2 are placed in a tumbler which is agitated or rotated. The sawdust or granular material is sprinkled over the pellets having the glue applied thereto so that the casing or coating 3 is gradually built up.

At this time or subsequently, the sky rocket sticks 4 may be applied in any desired manner. The adhesive character of the coating or casing 50 55 55 may be utilized to cause the stick to adhere.

The resultant fireworks article is ignited by means of a fuse 5 which is inserted through the port 6 of the casing or coating 3, a similar port 7 in the coating 2, and into a receiving opening 8 in the pellet 1.

5 This molded pellet 1, when ignited, produces sparks and flames and generates gases, the exit of which, through the opening through which the fuse 5 as been inserted, either tends to bring the article upright or to cause its flight as in the case of a sky rocket.

10 It will be understood that the exact composition of the pyrotechnic pellet 1 may be varied both as to the materials and colors produced and 15 may be utilized either to produce smoke alone or in combination with sparks or colors. Likewise, the conglomerated and agglomerated casing or covering 3 may be of any desired material.

15 Figures 11 to 14 inclusive illustrate a spinner embodying the features of this invention. When 20 a fuse is ignited, it causes the spinner to rotate and the wings 9 on the spinner will cause the entire body to elevate.

25 Figures 15 and 16 show a cylindrical body embodying this invention in the nature of a fountain which is adapted to hold its upright position when the fuse is ignited and the contents blow out of the fuse hole.

It will be understood that I desire to comprehend within my invention such modifications as come within the scope of the claims and the invention.

Having thus fully described my invention, what I claim as new and desire to secure by Letters Patent is:

1. In combination, a pressed pellet of pyrotechnic material and a coating consisting of silicate of soda, whiting and charcoal.

2. In combination, a pressed pellet of pyrotechnic material, a coating consisting of silicate of soda, whiting and charcoal, and a casing of agglomerated material.

3. In combination, a pressed pellet of pyrotechnic material, a coating consisting of silicate of soda, whiting and charcoal, and a casing of agglomerated material consisting of glue, and a filler such as sawdust and wood flour.

4. A sky rocket comprising a longitudinal pyrotechnic pellet having a fuse mounted in one end thereof, a coating of silicate of soda, whiting and charcoal on the pellet and an agglomerated casing of glue, and a filler and a stick attached to said casing.

ALBERTO CIMOROSI.